

1

2,974,002

MERCERIZING COMPOSITIONS CONTAINING  
PINONIC ACID

Glen W. Hedrick, Lake City, Fla., assignor to the United States of America as represented by the Secretary of Agriculture

No Drawing. Filed June 30, 1959, Ser. No. 824,156

1 Claim. (Cl. 8—125)

(Granted under Title 35, U.S. Code (1952), sec. 266)

10

A non-exclusive, irrevocable, royalty-free license in the invention herein described, throughout the world for all purposes of the United States Government, with the power to grant sublicenses for such purposes, is hereby granted to the Government of the United States of America.

This invention relates to the mercerization of cotton. More particularly, this invention relates to novel mercerizing compositions containing pinonic acid.

Mercerization is a widely used process wherein cotton, in the form of yarn or fabric, is treated under tension with strong caustic soda solution and then, while still under tension, is washed until the cotton is free of caustic. The mercerization treatment, as usually practiced, so alters the cotton that it has greater smoothness, a permanent luster, improved dye affinity and chemical reactivity, and increased tensile strength. If no tension is applied to the cotton during the treatment with the strong caustic, the cotton will shrink considerably and, upon washing, will show both greatly increased strength and dye affinity, but no luster.

The majority of practical mercerizations are carried out using caustic concentrations between 22 and 25%, but caustic strengths ranging from about 14 to 28% may be used. In conjunction with the strong caustic solution, it is generally desirable to use a wetting agent or so-called "mercerizing penetrant." The mercerizing penetrant dissolved in the caustic increases tremendously its penetrating power and helps to effect rapid and even wetting of the cotton with the caustic. Rapid, uniform, and efficient mercerization of the cotton is thereby made possible.

Most ordinary wetting agents cannot be used in the mercerizing process as they are not sufficiently soluble in the strong caustic solutions. The conventional mercerizing penetrants are generally of two basic types, although numerous admixtures of types may be employed. One main group of penetrants is based on phenolic compounds, particularly cresylic acid (cresols), and the other group is based on noncresylic high alcohols. The wetting power of the penetrant is usually increased by the addition of water-miscible organic solvents, frequently alcohols. The cresylic acid-type penetrants are more satisfactory for general use than the noncresylic type, but they have certain disadvantages—namely, their odor is objectionable and they have irritating properties when in contact with the skin.

In general, mercerizing penetrants are employed at approximately 1% concentration, based on the volume of the mercerizing caustic solution. The amount of a good penetrant required for the maximum effect rarely exceeds 2%. Some of the penetrants used in the prior art have high wetting powers, but usually only over a rather narrow range of caustic concentrations. Other penetrants can be used over a wider range of caustic concentrations, but they have poorer wetting powers.

It is an object of the present invention to provide novel mercerizing compositions containing pinonic acid. It is a further object of the invention to provide mercerizing compositions which rapidly and uniformly wet cotton over a wide range of caustic concentrations and tempera-

2

tures. Another object is to provide mercerizing compositions whose mercerizing penetrants do not possess objectionable or skin-irritating properties.

It has been discovered that pinonic acid, a carboxylic acid derivable from turpentine and represented by the following formula



when mixed with butyl Cellosolve (i.e., 2-n-butoxyethanol) is an effective mercerizing penetrant. The pinonic acid-butyl Cellosolve penetrant incorporated into caustic soda solutions of mercerizing strength gives almost instantaneous wetting of cotton with the caustic over a wide range of caustic concentrations and temperatures. The mercerizing penetrants of the present invention do not possess the objectionable odors and skin-irritating properties of many of the penetrants commonly used in the prior art. They compare favorably in wetting properties with the cresylic acid-type mercerizing penetrants of the prior art.

The effectiveness of the pinonic acid mercerizing penetrant is quite surprising in view of the fact that other carboxylic acids having  $\text{C}_8$ ,  $\text{C}_{10}$ , and  $\text{C}_{12}$  carbon chains are not generally satisfactory for use as wetting agents in mercerizing compositions. The unique structure and properties of pinonic acid are probably responsible for its effectiveness. Pinonic acid, as shown in the above formula, is a  $\text{C}_{10}$  monobasic acid containing a carbonyl (ketone) group. It is capable of forming, in strong caustic solutions, a sodium salt of both the carboxylic acid and the enol form of the ketone. It is believed that the enol form is important and that a certain amount of the enol salt is necessary for proper wetting; otherwise, the acid, because of the common ion effect, would not have the desired solubility for effective wetting. Pinonic acid's effectiveness is undoubtedly due to a relationship of molecular weight, configuration, and solubility characteristics.

Pinonic acid suitable for use in the mercerizing compositions of the present invention can be conveniently obtained from alpha-pinene, a major constituent of gum turpentine, by oxidation with ozone or potassium permanganate, as is well-known to those familiar with naval stores products.

The mercerizing compositions of the present invention contain pinonic acid and butyl Cellosolve dissolved in caustic soda solutions of mercerizing strength, the pinonic acid being present in the mercerizing composition in from about 0.08 to 0.64 weight percent and the butyl Cellosolve being present in from about 0.72 to 0.16 weight percent, the lesser amounts of the butyl Cellosolve being employed with the greater amounts of the pinonic acid. It is generally preferred to mix the pinonic acid with the butyl Cellosolve, and then add the penetrant mixture to the caustic soda solution. The proportion of pinonic acid present in the pinonic acid-butyl Cellosolve penetrant mixture can be varied widely—from about 10 to 80 wt. percent of the mixture. The preferred penetrant mixture contains 50 wt. percent of pinonic acid and 50 wt. percent of butyl Cellosolve. The quantity of penetrant mixture added to the caustic soda solution can be varied considerably, depending on the composition of the particular penetrant mixture employed and the rapidity of wetting desired by the operator. In general, about 1 gram of penetrant mixture is preferred for each 100 ml. of caustic soda solution, but effective wetting of cotton can be achieved using as little as 0.25 or 0.5 g. of

the 50:50 mixture of pinonic acid and butyl Cellosolve for 100 ml. of caustic solution.

The concentration of the caustic soda solution used in the mercerizing compositions of the invention can be varied widely. It is generally preferred to employ a caustic concentration between about 255 and 315 g. of NaOH per liter of solution (i.e. about 21 to 25% NaOH). However, if the preferred penetrant mixture consisting of 50 wt. percent pinonic acid and 50 wt. percent butyl Cellosolve is employed, effective wetting can be achieved using caustic concentrations ranging from about 165 to 345 g. of NaOH per liter (14 to about 28% NaOH).

The mercerizing compositions of the present invention maintain their effectiveness for wetting cotton over a rather wide range of operating temperatures. Using the preferred 50:50 mixture of pinonic acid and butyl Cellosolve as the penetrant in the mercerizing composition, almost instantaneous wetting of cotton with the mercerizing composition is achieved at temperatures ranging from 26° to 75° C.

The following examples are illustrative of certain details of the invention.

#### Example 1

Mixtures of pinonic acid and butyl Cellosolve, of the compositions indicated in the following table, were prepared. Each mixture was tested for its effectiveness as a mercerizing penetrant (i.e., evaluated as a wetting agent for cotton yarn in caustic soda of mercerizing concentration) in accordance with tentative test method 43-1952, "Evaluation of Penetrants for Mercerization," of the American Association of Textile Chemists and Colorists (1957 Technical Manual and Year Book of the American Association of Textile Chemists and Colorists, XXXIII, p. 156, Howes Publishing Co., Inc., New York, 1957). All tests were performed at a temperature of 26° C., using caustic concentrations of 285 grams of NaOH per liter of solution.

The data in the following table show the variations of wetting times of the cotton yarn samples with the various pinonic acid-butyl Cellosolve mixtures.

| Composition of Mercerizing Penetrant |                               | Wetting time seconds |
|--------------------------------------|-------------------------------|----------------------|
| Pinonic acid, wt. percent            | Butyl Cellosolve, wt. percent |                      |
| 10                                   | 90                            | 1.6                  |
| 20                                   | 80                            | 1.5                  |
| 30                                   | 70                            | 1.4                  |
| 40                                   | 60                            | 1.3                  |
| 50                                   | 50                            | 1.0                  |
| 60                                   | 40                            | 0.8                  |
| 70                                   | 30                            | 0.8                  |
| 80                                   | 20                            | 1.8                  |
| 100                                  | 0                             | >10                  |

#### Example 2

Mixtures of pinonic acid and butyl Cellosolve, and of cresylic acids and butyl Cellosolve, of the compositions indicated in the following table, were prepared. Each mixture was tested for its effectiveness as a mercerizing penetrant according to the procedure of Example 1. A standard, commercial mercerizing penetrant (a mixture of polyhydric alcohols and cresylate) was also tested for comparison. All tests were performed at a temperature of 26° C., using caustic concentrations of 285 grams of NaOH per liter of solution. The amount of penetrant used was varied as indicated in the following table.

The data in the table show the variations of wetting times of the cotton yarn samples with the mercerizing compositions containing the various kinds and concentrations of mercerizing penetrants.

| Mercerizing Penetrant No. | Composition of Mercerizing Penetrant    | Wetting time, seconds                    |     |      |      |       |
|---------------------------|-----------------------------------------|------------------------------------------|-----|------|------|-------|
|                           |                                         | g.1 or ml. penetrant for 100 ml. caustic |     |      |      |       |
|                           |                                         | 1.25                                     | 1   | 0.85 | 0.5  | 0.25  |
| 1.                        | Standard (Pinonic acid, 50 wt. percent) | 1.1                                      | 1.6 | 3.0  | 18.2 | ----- |
| 2.                        | Butyl Cellosolve, 50 wt. percent        | 1.3                                      | 1.4 | 1.6  | 2.1  | 2.9   |
| 3.                        | Pinonic acid, 75 wt. percent            | 1.0                                      | 1.1 | 1.5  | 14.6 | ----- |
| 4.                        | Butyl Cellosolve, 25 wt. percent        | 1.3                                      | 1.3 | 1.4  | 1.5  | 2.1   |
| 5.                        | Cresylic acids, 50 wt. percent          | 0.9                                      | 1.0 | 1.1  | 1.2  | 1.9   |
|                           | Butyl Cellosolve, 25 wt. percent        |                                          |     |      |      |       |

<sup>40</sup> <sup>1</sup> For mercerizing penetrants Nos. 2 and 3.

#### Example 3

A series of tests for effectiveness as mercerizing penetrants was conducted on the five mercerizing penetrant compositions of Example 2. In this series, one gram or milliliter of penetrant was used for 100 milliliters of caustic solution, and the caustic strength was varied from 50 165 to 465 grams of NaOH per liter of caustic solution. The other conditions of the tests were as previously described.

The data in the following table show the relative effectiveness of the various penetrants in the mercerizing compositions over the wide range of caustic concentrations.

| Mercerizing Penetrant No. | Composition of Mercerizing Penetrant | Wetting time, seconds                     |     |     |     |       |     |       |
|---------------------------|--------------------------------------|-------------------------------------------|-----|-----|-----|-------|-----|-------|
|                           |                                      | Caustic concentration, gms.NaOH per liter |     |     |     |       |     |       |
|                           |                                      | 165                                       | 225 | 255 | 285 | 315   | 345 | 465   |
| 1.                        | Standard                             | 8.5                                       | 1.7 | 1.5 | 2.5 | ----- |     |       |
| 2.                        | Pinonic acid, 50 wt. percent         | 2.2                                       | 0.7 | 0.9 | 1.5 | 1.7   | 2.7 | ----- |
| 3.                        | Butyl Cellosolve, 50 wt. percent     |                                           |     |     |     |       |     |       |
| 4.                        | Pinonic acid, 75 wt. percent         |                                           |     | 1.9 | 1.1 | 1.4   | 2.7 | ----- |
| 5.                        | Butyl Cellosolve, 25 wt. percent     |                                           |     |     |     |       |     |       |
| 4.                        | Cresylic acids, 50 wt. percent       | 1.6                                       | 0.8 | 1.1 | 1.4 | 1.9   | 2.3 | 8     |
| 5.                        | Butyl Cellosolve, 25 wt. percent     | 0.7                                       | 0.9 | 1.0 | 1.6 | 1.9   | 9   |       |

## Example 4

A series of tests for effectiveness as mercerizing penetrants was conducted on the five mercerizing penetrant compositions of Example 2. In this series, one gram of milliliter of penetrant was used for 100 milliliters of caustic solution. The caustic concentration was 285 grams of NaOH per liter of caustic solution. The tests were conducted at temperatures of 26°, 50° and 75° C. The other conditions of the tests were as previously described.

The data in the following table show the relative effectiveness of the five penetrants in the mercerizing compositions at the various temperatures.

| Mercerizing Penetrant No. | Composition of Mercerizing Penetrant                                           | Wetting time, seconds |     |     |
|---------------------------|--------------------------------------------------------------------------------|-----------------------|-----|-----|
|                           |                                                                                | Temperature, ° C.     |     |     |
|                           |                                                                                | 26                    | 50  | 75  |
| 1.....                    | Standard.....                                                                  | 1.7                   | 3.7 | >10 |
| 2.....                    | {Pinonic acid, 50 wt. percent.....<br>{Butyl Cellosolve, 50 wt. percent.....   | 1.5                   | 1.0 | 1.0 |
| 3.....                    | {Pinonic acid, 75 wt. percent.....<br>{Butyl Cellosolve, 25 wt. percent.....   | 1.1                   | 2.6 | 9.2 |
| 4.....                    | {Cresylic acids, 50 wt. percent.....<br>{Butyl Cellosolve, 50 wt. percent..... | 1.4                   | 1.3 | 1.4 |
| 5.....                    | {Cresylic acids, 75 wt. percent.....<br>{Butyl Cellosolve, 25 wt. percent..... | 1.0                   | 0.7 | 0.7 |

## I claim:

A mercerizing composition comprising an aqueous caustic soda solution of mercerizing strength, from about 0.08 to 0.64 weight percent of pinonic acid, and from about 0.72 to 0.16 weight percent of butyl Cellosolve, the lesser amounts of butyl Cellosolve being employed with the greater amounts of pinonic acid.

10

## References Cited in the file of this patent

## UNITED STATES PATENTS

|           |               |               |
|-----------|---------------|---------------|
| 2,679,509 | Hasselstrom   | May 25, 1954  |
| 2,750,411 | Fisher et al. | June 12, 1956 |
| 2,751,278 | Reeves et al. | June 19, 1956 |

15

## FOREIGN PATENTS

|         |               |              |
|---------|---------------|--------------|
| 734,749 | Great Britain | Aug. 3, 1955 |
|---------|---------------|--------------|

20

## OTHER REFERENCES

Summers et al.: American Dyestuff Reporter, vol. 47, pp. 571-573, August 25, 1958.